# EUROPEAN PATENT SPECIFICATION

(11) **EP 2 074 236 B1**
(45) Date of publication and mention of the grant of the patent: **20.02.2013**
(21) Application number: 07804280.1
(22) Date of filing: 12.09.2007
(51) Int. Cl.: C22C 23/06

(54) **MAGNESIUM GADOLINIUM ALLOYS**
MAGNESIUM-GADOLINIUM-LEGIERUNGEN
ALLIAGES DE MAGNÉSIUM ET DE GADOLINIUM

(30) Priority: 13.09.2006 GB 0617970
(43) Date of publication of application: 01.07.2009
(73) Proprietor: Magnesium Elektron Limited, Salford M50 3XE (GB)
(72) Inventor: WILKS, Timothy, E., Bury BL0 0AN (GB); JEREMIC, Sarka, Cheshire SK9 2QD (GB); ROGERS, Phillip, David, Manchester M28 1UT (GB); LYON, Paul, Bolton BL7 9RL (GB)
(74) Representative: Wise, Stephen James
(86) International application number: PCT/GB2007/003491
(87) International publication number: WO 2008/032087

(56) References cited:
- CN-A- 1 804 083
- JP-A- 9 263 871
- JP-A- 10 147 830
- SU-A1- 1 010 880
- YAMADA, KENTARO ET AL: "Precipitate microstructures of high strength Mg-Gd-Y- Zn - Zr alloys" ADVANCED MATERIALS RESEARCH (ZUERICH, SWITZERLAND) , 11-12(AICAM 2005), 417-420 CODEN: AMREFI; ISSN: 1022-6680, 2006, XP009092939
- HONMA, T. ET AL: "Effect of Zn additions on the age-hardening of Mg-2.0Gd-1.2Y-0.2Zr alloys" ACTA MATERIALIA , 55(12), 4137-4150 CODEN: ACMAFD; ISSN: 1359-6454, 2007, XP002462033
- LI, J. P. ET AL: "Microstructures of extruded Mg-12Gd-1Zn-0.5Zr and Mg-12Gd-4Y-1Zn-0.5Zr alloys" SCRIPTA MATERIALIA , VOLUME DATE 2007, 56(2), 137-140 CODEN: SCMAF7; ISSN: 1359-6462, 2006, XP002462034
- DATABASE WPI Derwent Publications Ltd., London, GB; AN 2006-069928 XP002471295 -& CN 1 676 646 A (UNIV SHANGHAI JIAOTONG [CN]) 5 October 2005 (2005-10-05) cited in the application
- DATABASE CA [Online] CHEMICAL ABSTRACTS SERVICE, COLUMBUS, OHIO, US; 4 December 2007 (2007-12-04), ZHANG, KUI ET AL: "Creep resistance Mg alloy and its manufacture" XP002471294 retrieved from STN Database accession no. 2007:1375313 -& CN 101 078 080 A (GENERAL RESEARCH INSTITUTE FOR NONFERROUS METALS, PEOP. REP. CHINA) 28 November 2007 (2007-11-28)

## Description

This invention relates to gadolinium-containing magnesium alloys, particularly those which possess high strength combined with corrosion resistance, and an optimised balance of strength and ductility. The described alloys also have exceptional high temperature performance for magnesium alloys. The alloys of the present invention have been developed as extrusion alloys, but can be rolled to produce sheets and are also suitable for forging and machining. Although they can be cast successfully to form billets, these alloys are not as suitable to use as shape casting alloys in processes such as die casting or sand casting as other magnesium alloys due to a tendency to form cracks.

There is considerable prior art concerning the Mg-Y-Gd system.

The United States patent US3391034 teaches that binary alloys of magnesium and 8 to 11wt% yttrium can be produced that are age-hardenable.

It states that the ductility of these alloys is inversely proportional to their yield strength, and that an acceptable ductility is greater than 3-5%. It teaches that for the magnesium yttrium system levels of yttrium less than 8wt% do not produce sufficient mechanical properties compared with other magnesium alloys.

The mechanical properties claimed in US3391034 are shown in Table 1.

**Table 1**

| Yttrium Content (wt%) | Yield Stress (Mpa) | UTS (Mpa) | Elongation % |
|---|---|---|---|
| 8.2 | 303 | 344 | 3 |
| 9.0 | 323 | 374 | 6 |
| 10.6 | 335 | 374 | 5 |

The Russian patent SU1010880 teaches about magnesium alloys containing yttrium and gadolinium, optionally with zirconium. The two specific alloys discussed in the patent specification have the mechanical properties summarised in Table 2.

**Table 2**

| Alloy Composition (wt%) | Yield Stress (MPa) | UTS (MPa) | Elongation (%) |
|---|---|---|---|
| 4-6% Y, 8-10% Gd, 0.3-1.0% Mn | 378-390 | 393-442 | 4.4-9.8 |
| 5-6.5% Y, 3.5-5.5% Gd, 0.15-0.7% Zr | 353-387 | 397-436 | 4.0-6.0 |

This prior art teaches that these types of manganese-containing alloy form cracks while casting, but that this effect is reduced by the replacement of the manganese with zirconium. This teaching is silent regarding the corrosion behaviour or isotropy of these alloys.

The Japanese patent JP10147830 teaches that an alloy containing 1-<6 wt% Gd and 6-12 wt% Y produces good strength at high temperature. Zirconium in an amount of up to 2 wt% can also be present.

Also the Japanese patent JP9263871 teaches that an alloy containing 0.8-5 wt% Y and 4-15 wt% Gd or Dy produces a product that can be forged to produce an alloy of good strength. There is however no recognition in this document of the importance of not only the amount of each alloying element but their respective ratios.

Using peak hardness as a measure some tests were carried out on alloys with constant values of atomic percent rare earths (Total Rare Earths), while varying the ratio of yttrium plus other soluble lanthanides to gadolinium. The results are as follows:

| Melt Number | At%Gd | At% Y+ other soluble lanthanides | At% TRE | Ratio of Y + other soluble lanthanides to Gd | Wt% Gd | Wt%Y+ Other soluble lanthanides | Peak Hardness (Hv) |
|---|---|---|---|---|---|---|---|
| DF9122 | 1.33 | 2.00 | 3.33 | 1.5 | 7.6 | 6.5 | 127 |
| DF9123 | 0.83 | 2.50 | 3.33 | 3.0 | 4.8 | 8.2 | 110 |
| DF9124 | 2.50 | 0.83 | 3.33 | 0.3 | 13.1 | 2.6 | 118 |

JP9263871 also discusses the addition of Ca and other lanthanides, but we have found that the addition of Ca and certain lanthanides is very deleterious to these types of alloys.

The Chinese patent CN1676646 purports to teach that a broad range of alloys containing 1-6 wt% Y, 6-15wt% Gd, 0.35-0.8 wt% Zr and 0-1.5 wt% Ca can be extruded to produce extrudates of good strength, but there is little specific description of the alloys of the Examples and no clear demonstration of the utility of the described alloys near the limits of the claimed range.

All this prior art seems to be focussed on maximising the strength of the alloy at the expense of its ductility, but this latter is an equally important material property. Furthermore there is no recognition in the prior art of the effect of the levels of the different alloying element on the corrosion behaviour of the described alloys. What the present invention teaches is a way to obtain improved ductility while also achieving high strength levels, without sacrificing corrosion resistance. None of this prior art recognises that when two or more of lanthanides and yttrium are in the same alloy, it is the specific ratio of their atomic concentrations that is the key factor in the effectiveness of the additions.

By selecting alloying additions within the range claimed in this invention and controlling the isotropy of the alloy, in addition to these improved mechanical properties, the alloys of the present invention will generally have corrosion rates of less than 100 mils per year (mpy) in the industry standard ASTM B117 salt-fog test, and preferably less than 50 mpy. Since the above prior art does not mention the corrosion performance of the described alloys and so it can be assumed that this feature of the described alloys was in line with conventional alloys, i.e. inferior to that of the alloys of the present invention and greater than a corrosion rate of 50 mpy.

In particular, in the academic published work by Rokhlin, namely the book entitled "Magnesium Alloys Containing Rare Earth Metals" Rokhlin, L L, published 2003, the inventor of SU1010880 states that increasing the yttrium content of magnesium alloys is detrimental to the corrosion rate of the alloy as shown in Table 3. The text states that this is due to the presence of Mg₂₄Y₅ compounds which are cathodic to the solid solution.

**Table 3**

| Yttrium Content | Corrosion Rate | |
|---|---|---|
| Wt% | mg/cm²/hour | Mills/years |
| 0.5 | 0.025 | 48 |
| 3.8 | 0.14 | 268 |
| 10.5 | 0.36 | 690 |

The invention is given in the claims.

In this specification soluble heavy lanthanides are defined as elements with atomic numbers 65 to 69 inclusive and 71. Soluble heavy lanthanides (SHL) are those which display substantial solid solubility in magnesium. They are terbium, dysprosium, holmium, erbium, thulium and lutetium. These elements are characterised by all of them having the same hexagonal close packed metallic structure as possessed by yttrium and magnesium, and by having a metallic radius of between 0.178nm and 0.173nm. They also exist only in a trivalent state when oxidised, which thus distinguishes them from elements such as europium and ytterbium which show both tri- and bivalency and do not show any appreciable solid solubility in magnesium. When present the aggregate level of soluble heavy lanthanides should be greater than 0.1 at% in order ot contribute significantly to the mechanical properties of the alloy. A particularly preferred soluble heavy lanthanide is erbium.

It is well known that the strengthening of alloys by precipitation hardening is a function of the amount and type of particles that are formed. This effect is related to both the amount of alloying elements that can be dissolved in the matrix expressed as atomic percent and not as weight percent, and to the potential to precipitate intermetallic particles by heat treatment. The binary phase diagrams for the soluble heavy lanthanides and magnesium, for yttrium and magnesium, and for gadolinium and magnesium all show this potential. From these phase diagrams it has been assumed to date that the soluble heavy lanthanides, gadolinium and yttrium will all strengthen magnesium in similar ways. It has, however, surprisingly been found that when gadolinium is present in a specific amount the addition of a soluble heavy lanthanide or yttrium within a defined range causes the formation of at least one indeterminate ternary phase which affects the alloy's mechanical properties. This at least one ternary phase requires a ratio between the soluble heavy lanthanide or yttrium and gadolinium of 3:2. Alloys having this ratio demonstrate a better combination of mechanical properties, namely strength, ductility and transverse properties, than can be achieved using other combinations of amounts of the lanthanides, yttrium and gadolinium. Significantly improved properties can be found where the ratio is between 1.25:1 and 1.75:1 for alloys which contain from 2.3 to 4.6 at% in total of gadolinium and at least one of soluble heavy lanthanide or yttrium. Outside this range either the strength and/or the ductility of the alloys declines. This decline becomes noticeable when the total amount of gadolinium, soluble heavy lanthanide and yttrium is below 2.0 at% and above 5.0 at%.

In order to assist this precipitation hardening effect a grain refining element can be added in an amount up to its solid solubility limit in the alloy. A preferred such element is zirconium. This can be added with increasing amounts generally improving the alloy's yield stress and elongation-to-failure properties. For such an effect at least 0.03 atomic per cent of zirconium should be present, and the maximum amount is the solid solubility limit of Zr in the alloy which is generally at about 0.3 atomic percent. However with both high and low levels of zirconium corrosion resistance may decline. The most preferred composition for a zirconium containing alloy of the present invention is 5.5 to 6.5 wt% Y, 6.5 to 7.5 wt% Gd and 0.2 to 0.4 wt% Zr, with the remainder being magnesium and incidental impurities. For some alloy compositions the level of zirconium should be from 0.3 to below 0.35% by weight in order to pass the 50 mpy salt-fog test.

It has been found that the presence of small amounts of zinc are beneficial to the corrosion performance of the alloys of the present invention, but that as the level of zinc is increased the alloy's corrosion performance deteriorates. Preferably the level of zinc should be from 0.07 to below 0.5at%. There also appears to be a linkage regarding the formation of different types of precipitates when both zirconium and zinc are present in the alloy, and it has been found that the ratio of zinc to zirconium should not exceed 2:1, and should be preferably less than 0.75:1.

Any lanthanide other than the required soluble heavy lanthanide or yttrium should be present in a total amount of less than 0.2 atomic per cent, and preferably below 0.1 at%, otherwise there is interference with the formation of the desired at least one indeterminate ternary phase as described above. Similarly any other element should be present in an amount of no more than 0.2 at%, preferably no more than 0.1 at%, and more preferably be present only at an incidental impurity level.

The alloys of the present invention may be used for extrusions, sheet, plate and forgings. Additionally they may be used for parts machined and/or manufactured from extrusions, sheet, plate or forgings.

### Examples

A magnesium alloy DF8791 was produced containing 3.04 at % in total of yttrium and gadolinium, where the yttrium to gadolinium ratio was 1.52:1. Additionally it contained 0.15 at% zirconium, with other elements being at impurity levels.

Another magnesium alloy, DF8961, was produced containing 2.65 at% in total of yttrium and gadolinium, with an yttrium to gadolinium ratio of 1.46:1. Additionally, it contained 0.12 at% Zr and 0.08 at% Zn, with other elements being at impurity levels.

Another magnesium alloy DF9380 was produced containing a a 3.03 at% of a mixture of erbium, gadolinium and yttrium with a soluble rare earth plus yttrium to gadolinium ratio of 1.38:1. Additionally it contained 0.125 at% zirconium.

All these alloys possessed yield stresses greater than 300MPa and elongations-to-failure greater than or equal to 10%.

Three further magnesium alloys were tested, namely alloys DF8915, DF9386 and DF8758, which had similar total levels of yttrium and gadolinium to those of DF8961 but in different ratios. DF8915 had a significantly higher ratio of 3.9:1 and this produced a reduced yield stress of only 250MPa. DF9386 and DF8758 both had a significantly lower ratio of 0.72:1 and 0.93:1 respectively. These low ratios had the effect of reducing the ductility of these alloys to below 5% to levels that are commercially unacceptable for this type of product.

A further alloy magnesium alloy DF9381 was produced containing 2.99 at% of a mixture of ytterbium, gadolinium and yttrium with a soluble rare earth plus yttrium to gadolinium ratio of 1.39:1. Additionally it contained 0.121 at% zirconium. The ytterbium in this alloy is not a soluble heavy lanthanide, and as a result of its addition to the alloy the strength of the alloy was reduced to unacceptably low levels.

A further set of test alloys were produced to examine the effect of zirconium on corrosion for the alloys of the present invention. Melts DF9382a to DF9382e all had the same composition except for varying levels of zirconium. Alloy DF9382a shows that if the material is zirconium free (i.e. below detectable limits with standard industrial spark emission spectroscopy) the corrosion rate is above the acceptable level of 50 mils per year corrosion in the standard salt fog test. Further, at higher levels of zirconium for this alloy, DF9382b and DF9382c also show this poor behaviour. However at levels of zirconium between 0.03 at % (0.1 wt %) and 0.12 at % (0.4 wt%) good corrosion performance is achieved. This is demonstrated by DF9382d and DF9382e.

A summary of these test results is shown in Table 4, in which some of the data has been rounded.

**Table 4**

| Melt No | Analysis | | | | | | | | | | Tensile Properties | | | Corrosion |
|---|---|---|---|---|---|---|---|---|---|---|---|---|---|---|
| | Y | | Others | | Gd | | Zr | | Total HL+Y+Gd | HL+Y: Gd | 0.2% MPa | UTS MPa | %El | MPY |
| | Wt% | At % | Wt % | At % | Wt % | At % | Wt % | At % | | | | | | |
| DF8791 | 6 | 1.83 | | | 7 | 1.21 | 0.5 | 0.15 | 3.04 | 1.52 | 317 | 444 | 10 | |
| DF8961 | 5.2 | 1.57 | Zn 0.2 | Zn 0.08 | 6.3 | 1.08 | 0.4 | 0.12 | 2.65 | 1.46 | 308 | 424 | 17 | |
| DF9380 | 5.09 | 1.55 | Er 0.94 | Er 0.15 | 7.72 | 1.33 | 0.42 | 0.125 | 3.03 | 1.38 | 306 | 409 | 13 | |
| DF8915 | 8.1 | 2.44 | | | 3.7 | 0.63 | 0.5 | *0.15* | 3.07 | 3.9 | 250 | 356 | 13 | |
| DF9386 | 5.13 | 1.64 | | | 12.64 | 2.29 | 0.24 | 0.075 | 3.93 | 0.72 | 359 | 450 | 3.5 | |
| DF8758 | 4.7 | 1.45 | | | 8.9 | 1.55 | 0.4 | 0.12 | 3.0 | 0.93 | 319 | 433 | 3.9 | |
| DF9381 | 5.18 | 1.58 | Yb 1.0 | Yb 0.16 | 7.28 | 1.25 | 0.41 | 0.121 | 2.99 | 1.39 | 264 | 367 | 15 | |
| | | | | | | | | | | | | | | |
| DF9382a | 6 | 1.83 | | | 7 | 1.21 | 0 | 0 | 3.04 | 1.52 | | | | 58 |
| DF9382b | 6 | 1.83 | | | 7 | 121 | 0.41 | 0.13 | 3.04 | 1.52 | | | | 58 |
| DF9382c | 6 | 1.83 | | | 7 | 1.21 | 0.5 | 0.147 | 3.04 | 1.52 | | | | 285 |
| DF9382d | 6 | 1.83 | | | 7 | 1.21 | 0.33 | 0.098 | 3.04 | 1.52 | | | | 17 |
| DF9382e | 6 | 1.83 | | | 7 | 1.21 | 0.24 | 0.071 | 3.04 | 1.52 | | | | 9 |

## Claims

1. A magnesium alloy consisting of:
2.0 to 5.0 at% in total of gadolinium and at least one element selected from the group consisting of soluble heavy lanthanides and yttrium, wherein the soluble heavy lanthanides are terbium, dysprosium, holmium, erbium, thulium and lutetium, and wherein the ratio of the aggregate amount of soluble heavy lanthanides and yttrium to the amount of gadolinium is between 1.25:1 and 1.75:1,
all other lanthanides in an aggregate amount of less than 0.2 at%,
optionally zinc in an amount of from 0.06 to 0.6 at%, and
the balance being magnesium, with any other element being present only as an incidental impurity in an amount of less than 0.2 at%;
**characterised in that** the alloy additionally contains zirconium in an amount of from 0.06 to 0.12 at%.

2. An alloy as claimed in claim 1 wherein the total amount of gadolinium, at least one soluble heavy lanthanide and yttrium is 2.3 to 4.6 at%.

3. An alloy as claimed in claim 1 or claim 2 wherein the said ratio is approximately 1.5:1.

4. An alloy as claimed in any one of claims 1 to 3 wherein at least one soluble heavy lanthanide is present in an amount of at least 0.1 at%.

5. An alloy as claimed in claim 4 wherein the at least one soluble heavy lanthanide is erbium.

6. An alloy as claimed in any one of the preceding claims wherein all other lanthanides are present in an aggregate amount of less than 0.1 at%.

7. An alloy as claimed in any one of the preceding claims wherein any other element is present in the amount of less than 0.1 at%.

8. An alloy as claimed in any one of the preceding claims additionally containing zinc in an amount of from 0.06 to 0.6 at%.

9. An alloy as claimed in claim 8 wherein zinc is present in an amount of from 0.07 to less than 0.5at%.

10. An alloy as claimed in any one of the preceding claims additionally containing a grain refining element in an amount up to its solid solubility limit in the alloy.

11. An alloy as claimed in claim 1 wherein zirconium is present in an amount of from 0.06 to 0.1 at%.

12. An alloy as claimed in claim 1 or claim 11 additionally containing zinc wherein the amount of zinc is such that the ratio of the weight of zinc to the weight of zirconium is less than 2:1.

13. An alloy as claimed in claim 12 wherein the zinc/zirconium ratio is less than 0.75:1.

14. An alloy as claimed in any one of the preceding claims having a corrosion rate less than 50 mils per year in a standard salt-fog test.

15. An alloy as claimed in claim 1 consisting of 5.5-6.5 wt% Y, 6.5- 7.5 wt% Gd and 0.2-0.4 wt% Zr with the remainder being magnesium and incidental impurities.

16. An alloy as claimed in claim 15 containing 0.3 to 0.35 wt% Zr.

17. An alloy as claimed in any one of the preceding claims when wrought and in the form of an extrusion, sheet, plate forging or mechanical part.

18. An alloy as claimed in claim 15 or claim 16 having a corrosion rate less than 50 mils per year in a standard salt-fog test.

## Patentansprüche

1. Eine Magnesiumlegierung, die aus Folgendem besteht:
insgesamt 2,0 bis 5,0 At% an Gadolinium und mindestens einem Element, ausgewählt aus der Gruppe, bestehend aus löslichen schweren Lanthaniden und Yttrium, wobei die löslichen schweren Lanthanide Terbium, Dysprosium, Holmium, Erbium, Thulium und Lutetium sind, und wobei das Verhältnis der Gesamtmenge an löslichen schweren Lanthaniden und Yttrium zu der Menge an Gadolinium zwischen 1,25:1 und 1,75:1 1 beträgt,
alle anderen Lanthanide in einer Gesamtmenge von weniger als 0,2 At%,
optional Zink in einer Menge von von 0,06 bis 0,6 At%, und
wobei der Rest Magnesium ist, wobei jedes beliebige andere Element lediglich als ein Nebenfremdstoff in einer Menge von weniger als 0,2 At% vorhanden ist;
**dadurch gekennzeichnet, dass** die Legierung zusätzlich Zirconium in einer Menge von von 0,06 bis 0,12 At% enthält.

2. Legierung gemäß Anspruch 1, wobei die gesamte Menge an Gadolinium, mindestens einem löslichen schweren Lanthanid und Yttrium 2,3 bis 4,6 At% beträgt.

3. Legierung gemäß Anspruch 1 oder Anspruch 2, wobei das besagte Verhältnis ungefähr 1,5:1 beträgt.

4. Legierung gemäß einem der Ansprüche 1 bis 3, wobei mindestens ein lösliches schweres Lanthanid in einer Menge von mindestens 0,1 At% vorhanden ist.

5. Legierung gemäß Anspruch 4, wobei das mindestens eine lösliche schwere Lanthanid Erbium ist.

6. Legierung gemäß einem der vorhergehenden Ansprüche, wobei alle anderen Lanthanide in einer Gesamtmenge von weniger als 0,1 At% vorhanden sind.

7. Legierung gemäß einem der vorhergehenden Ansprüche, wobei jedes beliebige andere Element in einer Menge von weniger als 0,1 At% vorhanden ist.

8. Legierung gemäß einem der vorhergehenden Ansprüche, die zusätzlich Zink in einer Menge von von 0,06 bis 0,6 At% enthält.

9. Legierung gemäß Anspruch 8, wobei Zink in einer Menge von von 0,07 bis weniger als 0,5 At% vorhanden ist.

10. Legierung gemäß einem der vorhergehenden Ansprüche, die zusätzlich ein Kornfeinungselement in einer Menge von bis zu seiner Festlöslichkeitsgrenze in der Legierung enthält.

11. Legierung gemäß Anspruch 1, wobei Zirconium in einer Menge von von 0,06 bis 0,1 At% vorhanden ist.

12. Legierung gemäß Anspruch 1 oder Anspruch 11, die zusätzlich Zink enthält, wobei die Menge an Zink so ist, dass das Verhältnis des Gewichts an Zink zu dem Gewicht an Zirconium weniger als 2:1 beträgt.

13. Legierung gemäß Anspruch 12, wobei das Zink/Zirconium-Verhältnis weniger als 0,75:1 beträgt.

14. Legierung gemäß einem der vorhergehenden Ansprüche mit einer Korrosionsrate von weniger als 50 mil pro Jahr in einem Standardsalzsprühnebeltest.

15. Legierung gemäß Anspruch 1, die aus 5,5-6,5 Gew.-% Y, 6,5-7,5 Gew.-% Gd und 0,2-0,4 Gew.-% Zr besteht, wobei der restliche Teil Magnesium und Nebenfremdstoffe sind.

16. Legierung gemäß Anspruch 15, die 0,3 bis 0,35 Gew.-% Zr enthält.

17. Legierung gemäß einem der vorhergehenden Ansprüche, wenn bearbeitet und in der Form einer Extrusion, eines Blechs, eines Plattenschmiedestücks oder eines mechanischen Teils.

18. Legierung gemäß Anspruch 15 oder Anspruch 16 mit einer Korrosionsrate von weniger als 50 mil pro Jahr in einem Standardsalzsprühnebeltest.

## Revendications

1. Un alliage de magnésium consistant en :
de 2,0 à 5,0 at% en totalité de gadolinium et au moins un élément sélectionné dans le groupe consistant en lanthanides lourds solubles et yttrium, dans lequel les lanthanides lourds solubles sont le terbium, le dysprosium, l'holmium, l'erbium, le thulium et le lutétium, et dans lequel le rapport entre la quantité d'agrégat de lanthanides lourds solubles et d'yttrium et la quantité de gadolinium est entre 1,25/1 et 1,75/1,
tous les autres lanthanides dans une quantité d'agrégat inférieure à 0,2 at%, facultativement du zinc dans une quantité allant de 0,06 à 0,6 at%, et
le reste étant du magnésium, tout autre élément étant présent seulement comme impureté imprévue dans une quantité inférieure à 0,2 at% ;
**caractérisé en ce que** l'alliage contient additionnellement du zirconium dans une quantité allant de 0,06 à 0,12 at%.

2. Un alliage tel que revendiqué dans la revendication 1 dans lequel la quantité totale de gadolinium, d'au moins un lanthanide lourd soluble et d'yttrium va de 2,3 à 4,6 at%.

3. Un alliage tel que revendiqué dans la revendication 1 ou la revendication 2 dans lequel ledit rapport est approximativement de 1,5/1.

4. Un alliage tel que revendiqué dans une quelconque des revendications 1 à 3 dans lequel au moins un lanthanide lourd soluble est présent dans une quantité d'au moins 0,1 at%.

5. Un alliage tel que revendiqué dans la revendication 4 dans lequel cet au moins un lanthanide lourd soluble est de l'erbium.

6. Un alliage tel que revendiqué dans une quelconque des revendications précédentes dans lequel tous les autres lanthanides sont présents dans une quantité d'agrégat inférieure à 0,1 at%.

7. Un alliage tel que revendiqué dans une quelconque des revendications précédentes dans lequel tout autre élément est présent dans la quantité inférieure à 0,1 at%.

8. Un alliage tel que revendiqué dans une quelconque des revendications précédentes contenant additionnellement du zinc dans quantité allant de 0,06 à 0,6 at%.

9. Un alliage tel que revendiqué dans la revendication 8 dans lequel le zinc est présent dans une quantité allant de 0,07 à moins de 0,5 at%.

10. Un alliage tel que revendiqué dans une quelconque des revendications précédentes contenant additionnellement un élément d'affinage du grain dans une quantité allant jusqu'à sa limite de solubilité à l'état solide dans l'alliage.

11. Un alliage tel que revendiqué dans la revendication 1 dans lequel le zirconium est présent dans une quantité allant de 0,06 à 0,1 at%.

12. Un alliage tel que revendiqué dans la revendication 1 ou la revendication 11 contenant additionnellement du zinc dans lequel la quantité de zinc est telle que le rapport entre le poids du zinc et le poids du zirconium est inférieur à 2/1.

13. Un alliage tel que revendiqué dans la revendication 12 dans lequel le rapport zinc/zirconium est inférieur à 0,75/1.

14. Un alliage tel que revendiqué dans une quelconque des revendications précédentes ayant un taux de corrosion inférieur à 50 mils par an dans un test de brouillard salin standard.

15. Un alliage tel que revendiqué dans la revendication 1 consistant en de 5,5 à 6,5 % en poids de Y, de 6,5 à 7,5 % en poids de Gd et de 0,2 à 0,4 % en poids de Zr, ce qui reste étant du magnésium et des impuretés imprévues.

16. Un alliage tel que revendiqué dans la revendication 15 contenant de 0,3 à 0,35 % en poids de Zr.

17. Un alliage tel que revendiqué dans une quelconque des revendications précédentes lorsqu'il est travaillé et sous la forme d'une extrusion, d'une feuille, d'un forgeage en plaque ou d'une pièce mécanique.

18. Un alliage tel que revendiqué dans la revendication 15 ou la revendication 16 ayant un taux de corrosion inférieur à 50 mils par an dans un test de brouillard salin standard.
